

Jan. 31, 1928.

1,657,950

W. L. WRIGHT

CONTAINER CLOSURE DISK AND THE PRODUCTION AND APPLICATION THEREOF

Filed May 19, 1926

*Fig. 1.*



*Fig. 2.*



*Fig. 3.*



*W. L. Wright* <sup>Inventor</sup>

*By*

*Herbert E. Pek*

*Attorney*

## UNITED STATES PATENT OFFICE.

WILBUR L. WRIGHT, OF FULTON, NEW YORK, ASSIGNOR TO OSWEGO FALLS CORPORATION, OF FULTON, NEW YORK, A CORPORATION OF NEW YORK.

## CONTAINER-CLOSURE DISK AND THE PRODUCTION AND APPLICATION THEREOF.

Application filed May 19, 1926. Serial No. 110,272.

This invention relates to improvements in binder carrying fibrous material hood cap disks and the like and to the production and application thereof; and the objects and nature of the invention will be readily understood by those skilled in the art in the light of the following explanations of the method involved and of the accompanying drawings that illustrate what I now believe to be the preferred mechanical expression or embodiment of my invention from among other forms, materials, arrangements and combinations within the spirit and scope thereof.

An object of the invention is to provide, produce and apply a paper or like fibrous material hood cap (and by the term hood cap I include hood cap disks or disks to be formed into skirted hood cap form on or over the container head or mouth) that carries, at least in its annular skirt, an exceedingly strong binder of high melting point and quick cooling or setting properties, capable of rendering said skirt soft and moldable when highly heated for molding and contraction under the rim of a container head, and capable of causing said skirt to then quickly set to stiff permanent cap securing form under said rim, and imparting to said skirt the quality of stripping or peeling from the glass bottle surface without leaving on such surface an objectionable bottle fouling deposit that is not readily removed therefrom by bottle washing methods employed in bottling establishments or dairies, and to enable said cap to be repeatedly reheated and subjected to heating for an abnormal length of time without destroying or seriously deteriorating the holding or binding qualities of the binder or of the cap skirt, and to reduce to the minimum the cost of binder carrying hood caps.

With these and other objects in view my invention is based on and involves the method of producing and of applying a hood cap disk having at least a securing portion or band the fibrous material of which is internally provided with a solid structure or deposit constituting a binder and possessing the characteristics of sulphur and its equivalent or equivalents.

Referring to the accompanying drawings forming a part hereof:

Fig. 1 is an elevation of the head or mouth portion of a container, such as a glass milk

or other bottle having an exterior rim or annular enlargement, sealed or covered by a hood cap in accordance with my invention.

Fig. 2 shows the bottle head in elevation and the secured hood cap in section.

Fig. 3 is a detail elevation of a fibrous or paper material hood cap in accordance with my invention.

The drawings show the head or mouth portion of a container *a*, such as a glass milk bottle, having the exterior annular rim or enlargement that provides an annular downwardly facing abutment or shoulder *b*, contracting and merging into the container neck *c*.

The hood cap that I happen to show as an example is composed of flexible sheet paper, and I herein employ the term "paper" in a broad sense to cover and include all fibrous materials that are equivalents within my invention, for hood cap purposes and that meet the requirements of my invention. The hood cap, that I happen to show, is composed of a single flexible fibrous material sheet of one thickness, and is in the form of a skirted disk preferably imperforate throughout. The hood cap is drawn by suitable dies to provide a central elevated usually flat circular top 1, the top surface of which is preferably of a character to receive and display suitable advertising or other legends or indicia applied thereto by printing, lithography or other process, and an annular preferably downwardly and outwardly flaring skirt 2 which can be longer or much shorter than shown. The skirt can be just long enough to contract and lock under the rim or can be slightly longer to extend to or onto the bottle neck. The length of the skirt is not material provided it is of a length to insure a binder carrying securing portion to contract to rigid form under a rim or into a recess, for securing the cap on and covering the bottle mouth.

The dies in drawing the single ply paper sheet material into the skirted form, gather or take up the surplus material by crimps, gathers, tucks or otherwise extending longitudinally of the cap skirt, preferably in the form of overlapping tucks 4, arranged in an annular series surrounding the skirt. The dies in shaping the skirt and tucks apparently tend to loosen, crush or break down the internal fibrous structure of the paper

60

70

75

80

85

90

95

100

105

110

material of the skirt between the paper side faces, and thereby render the skirt peculiarly adapted to readily internally take up a maximum quantity of binder of the character hereinafter described.

10 The paper material hood cap is provided with an annular securing portion 3, consisting of binder material carried by an annular portion of paper impregnated with or by the binder, whether such portion of paper is formed by the cap skirt or by a separate paper ring surrounding the skirt of the cap to hold the same contracted when secured under the container rim.

15 The annular cap securing or binder carrying portion 3, is formed by introducing sulphur, or material or a composition having the characteristics of sulphur, for my purposes, into the body of the paper material 20 to constitute an impregnum or impregnums as distinguished from a mere surface coating, and to form within the paper one or more normally stiff comparatively strong internal structures or frameworks of solidified sulphur.

25 I prefer to employ refined or sublimated sulphur, as sulphur in the raw state contains a substantial proportion of earthy or foreign matter.

30 Sulphur has a high melting point, namely, about 237° F., (or depending on conditions somewhere between about 231° F. and about 246° F.) and is quick setting to a hard rigid condition, and because of these qualities, its 35 water resistant characteristics, its tensile strength, its desirable color, and its very low cost, is highly desirable as a hood cap binder. However, I have not heretofore been able to successfully use a hood cap carrying sulphur alone as the binding agent, because of the 40 brittleness of this product when cold and its consequent failure to adhere to the paper surface by reason of its tendency to crumble and flake therefrom, and because I had not 45 then discovered certain peculiar desirable hood cap binder characteristics of sulphur and certain desirable qualities thereof when sulphur is employed as a hood cap binder impregnum.

50 I have discovered that sulphur can be successfully employed as a binder, when solidified within the body of the paper that constitutes the securing portion of the hood cap. In order to drive the sulphur into the 55 fibrous mass of the body of the paper of the hood cap or of the annular paper securing portion thereof or therefor, I find it necessary to subject the hood caps that have been drenched with or exteriorly carry quantities 60 of melted sulphur, to a more or less prolonged heat treatment at a temperature higher than the melting point of sulphur.

65 For instance, I can arrange the paper hood caps, before the binder has been applied thereto, in piles or stacks, each stack con-

sisting of a suitable number of the paper caps nested together with their skirts extending in the same direction. I then drench the stacks of caps with the hot melted readily flowable sulphur, in such manner that the 70 desired quantities of the molten sulphur collect on and adhere to the annular exposed portions of the cap skirts and may travel along the skirts toward the cap tops and between the nested caps. However, I do not 75 wish to limit myself to any particular method of applying the liquefied melted sulphur to the cap skirts, as various means or methods can be used or followed for this purpose.

80 The melted sulphur for application to the hood cap skirts is preferably kept below the temperature at which the melted sulphur changes from the desirable light yellow color to a dark or reddish brown color. I prefer to apply the sulphur to the caps while it is 85 of the desirable light color.

Whatever method is followed in applying the light colored liquid sulphur to the caps, or if desired only to the cap skirts, so that 90 coatings of the hot liquid sulphur are retained on the caps, I subject the caps with the liquid sulphur thereon to a continued high temperature heat treatment in an oven or heating chamber, by which treatment I have been able to drive the liquid sulphur from the exterior of the paper into the interior of the paper caps or into the cap skirts to combination with the fibrous mass. This so-called 95 dewaxing treatment is continued until the cap, or the cap skirt is without free or exterior sulphur coatings and the securing portion of the cap skirt is approximately saturated with liquid sulphur.

100 For instance, I have attained the results sought by maintaining the paper caps carrying the liquid sulphur at a high temperature, say from about 275° F. to about 315° F. until the caps or the cap skirts have absorbed all 105 of the liquid sulphur deposited thereon, which result I accomplished by holding the 110 liquid-sulphur-drenched caps for about thirty minutes at said high temperature.

110 I find that the liquid sulphur is gradually absorbed by the cap skirts even at the high temperature and but slowly spreads within the cap skirts and that each cap skirt has 115 taken up and absorbed the desired quantity of sulphur needed to form the binder impregnum, before the liquid sulphur within the paper has spread to or into the flat top of the cap. It is desirable to keep the binder from the flat printed cap top for the sake of appearance and for reasons of economy in binder consumption.

120 When the cap skirts have absorbed the desired quantities of liquid sulphur to constitute the binder impregnums, the caps are allowed to cool and set. The sulphur even in the form of an impregnum within the paper, sets very quickly, without surface 125 130

coating of sulphur, and the hood caps are then ready for distribution and use. The caps carrying the binder impregnums, do not stick or adhere together, even when 5 nested.

These caps carrying the hard solidified binder impregnums, must be reheated at the bottling plant to render the skirts soft and moldable preparatory to application of the 10 caps to the containers and molding of the soft hot skirts to the bottle heads and contraction thereof under the bottle rims, by suitable clamping or molding heads. When thus molded against the cold glass surfaces, 15 the cap skirts quickly cool and set to hard stiff cap securing form and condition.

When desired, the hood caps thus secured, can be removed from the bottle heads by using the necessary force to tear or expand 20 the contracted annular securing portions of the cap skirts. The securing portions of the cap skirts will strip or peel from the glass bottle surfaces without fouling the same and without leaving objectionable binder 25 deposits thereon even should the securing or impregnated portion of the skirt have slightly adhering contact with the glass surface. The securing portion of the cap skirt is 30 without sufficient exterior binder coating to leave an objectionable fouling deposit on the glass even should the binder be when soft of a sticky or adhesive-to-glass nature. The securing portion of the skirt in any event 35 will strip or peel from the glass somewhat in the manner of surgical plaster.

At the plant while bottles are being hood capped, the hood caps of my invention to be applied, are kept in a suitable oven or heating chamber wherein the caps are subjected 40 to a temperature much higher than the melting point of the cap binder, and are taken from this oven and quickly applied. Where sulphur alone constitutes the cap binder, the caps to be applied are subjected to a temperature 45 approximately up to but preferably not above about 315° F. but always are kept below the high temperatures at which sulphur ignites and at which sulphur changes in character and color, and the caps 50 being thus prepared for application to the bottles, are not intended to be kept at this high temperature, even during temporary halts in the bottling and capping operations, for any extended length of time.

55 I have discovered that paper hood caps carrying binders consisting of sulphur impregnums, do not under repeated heat treatments lose their effective binding qualities by evaporation or otherwise and that the 60 sulphur does not so spread in the paper as to reduce the effective holding and binding strength of the cap securing portion. The sulphur when forming a hood cap binder, does not lose its desirable color and binding 65 qualities but is of a permanent nature,

and also has slow paper penetrating qualities which is desirable in preventing spread thereof onto the cap tops and in maintaining the concentration of the binder in the annular securing portion of the skirt, during 70 reheating of the caps for application.

While the drawings indicate by dotted or stippled surface 3<sup>a</sup>, the annular stiff hard securing portion of the cap that is impregnated with sulphur preferably to the 75 point of saturation forming what might be termed a stiff ring or frame of solidified sulphur and mass of fibers, yet I do not wish to limit my invention to any particular relative extent or location of said securing portion as any other annular portion of the skirt or the entire skirt might be so impregnated or even the entire cap.

80 Sulphur is an exceedingly plentiful and cheap product, even refined sulphur at present sells for about three cents per pound, as compared with other desirable plastic binders that I have heretofore used that run in cost from about twenty-five to fifty cents per pound. Furthermore sulphur renders 85 the paper to which applied of a very desirable color, paper impregnated therewith even when hot is not objectionably sticky and will strip or peel from glass when cold without objectionably fouling glass and 90 metal surfaces, is very quick setting, is of high melting point and hard and of great tensile strength particularly when permeated with and included within a fibrous mass, is not materially vaporized or reduced 95 in strength by repeated melting or reheating, is odorless in the cold state as when employed with cold bottled products, and paper impregnated thereby is rendered water-resistant and is water-proofed thereby. 100

105 It is understood of course that the entire cap can be impregnated with the binder without departing from my invention.

What I claim is:

110 1. A paper material hood cap, the skirt of which carries a sulphur binder impregnum solidified within the fibrous mass of the paper material and extending to the surfaces thereof and rendering the impregnated skirt 115 of the cap hard, water resistant, quick-setting, soft and moldable when heated above the melting point of the impregnum, and when either hot or cold non-fouling on glass bottle surfaces and capable of peeling or stripping therefrom.

120 125 2. An annularly-skirted hood cap composed of sheet paper the annular skirt of which is interiorly provided with a sulphur binder impregnum combined with the internal fibrous mass of the paper sheet rendering said binder carrying portion of the skirt capable of repeated heating to a temperature above the melting point of the binder without material loss of binding strength, said binder being of high-melting 130

point, quick-setting, and said impregnated portion of the skirt being non-fouling on and capable of stripping or peeling from container surfaces.

5. 3. An annularly skirted paper material hood cap carrying a binder embodying sulphur permanently carried by and incorporated in the cap skirt and rendering said skirt moldable when highly heated and 10 quick setting.

4. A fibrous material skirted hood cap provided with a binder composed of sulphur permanently incorporated therein, in combination with a container the head of which 15 is formed with an exterior shoulder, said cap covering said head with the skirt thereof molded under said shoulder and set to hard securing condition.

5. A fibrous material skirted hood cap, the 20 skirt of which is formed with an annular securing portion by the presence of sulphur solidified within and combined with the mass of fibers in said portion.

6. A fibrous material skirted hood cap 25 carrying a binder composed of a solidified impregnum of sulphur.

7. A fibrous material skirted hood cap having a securing portion carrying a binder 30 impregnum embodying sulphur driven into and solidified within the fibrous mass and extending to the surface thereof without substantial exposed surface coating rendering said portion capable of peeling or stripping 35 from glass surfaces without leaving fouling deposits thereon, said portion being hard and of substantial strength, quick-setting, water resistant, and capable of being

softened for molding by repeated high heating.

8. A paper material annularly skirted 40 hood cap carrying a solidified sulphur binder driven thereinto from the exterior thereof by continued heat substantially higher than the melting point of sulphur.

9. In the method of producing binder-45 carrying paper material hood caps and closing containers thereby, those steps which consist in externally applying sulphur liquefied by heat to a paper hood cap and maintaining such cap at a temperature substantially higher than the melting point of sulphur to drive the sulphur into the paper to form an impregnum therein, permitting the sulphur to set or solidify therein by cooling then softening the cap for molding 50 by heating the same to a temperature above the sulphur melting point, then applying the soft hot cap to the container head and molding the same thereto, and then allowing the 55 cap to set to rigid secured form.

10. In the production of binder carrying skirted hood caps, those steps which consist in applying sulphur exteriorly to the cap skirt and maintaining the same under high temperature substantially higher than the sulphur melting point until the sulphur has been absorbed by and taken into the paper to set therein and form an impregnum of solidified sulphur.

In testimony whereof, I have hereunto set 70 my hand at Fulton, New York, this 18th day of May, 1926.

WILBUR L. WRIGHT.